

# United States Patent Office.

JOHN MEEHAN, OF NEWARK, NEW JERSEY.

*Letters Patent No. 67,563, dated August 6, 1867.*

## IMPROVEMENT IN TANNING.

The Schedule referred to in these Letters Patent and making part of the same.

I, JOHN MEEHAN, of Newark, county of Essex, State of New Jersey, have discovered a process by which hemlock leather, after having been thoroughly tanned in hemlock barks or liquors, may be changed by my process to possess nearly all the qualities of leather tanned in liquors three-quarters oak and one-quarter hemlock.

I will first describe what I consider the best means of carrying out my invention, and will afterwards designate the points which I believe to be new.

To one part muriate of tin add two hundred and sixty parts of strong oak liquor, extracted about as follows: what tanners generally call a double liquor, that is, the extract of one leach pumped on to fresh bark and boiled about four hours, then allowed to cool down to a temperature of from 100° to 110°, the leather to be handled in that liquor for two and a half hours. If the desired effect be not produced in that length of time a very small proportion of the acid may be added, and the leather remain longer in, according to the judgment of the person using it.

Having now fully described my invention, what I claim as new, and desire to secure by Letters Patent, is—

The within-described process of changing hemlock leather so as to obtain in good part the qualities and appearance of oak-tanned leather, substantially as herein specified.

In testimony whereof I have hereunto set my hand in the presence of the subscribing witnesses.

JOHN MEEHAN.

Witnesses:

FRANCIS MEEHAN,

JOHN BRADY.